

## [54] COATING METHOD

[75] Inventors: **Yoshio Tanimoto; Tadamitsu Nakahama; Takakazu Yamane; Shunji Masuda**, all of Hiroshima, Japan

[73] Assignee: **Mazda Motor Corporation**, Hiroshima, Japan

[21] Appl. No.: 328,544

[22] Filed: Mar. 24, 1989

## [30] Foreign Application Priority Data

Mar. 25, 1988 [JP] Japan ..... 63-71337  
Mar. 25, 1988 [JP] Japan ..... 63-71339

[51] Int. Cl.<sup>5</sup> ..... B05D 3/06

[52] U.S. Cl. ..... 427/46; 427/55;

427/379; 427/388.2; 427/409; 427/425

[58] Field of Search ..... 427/46, 55, 379, 388.1, 427/388.2, 388.4, 388.5, 409, 425

## [56] References Cited

## U.S. PATENT DOCUMENTS

4,610,898 9/1986 Engel et al. ..... 427/388.4 X  
4,661,410 4/1987 Geist ..... 427/388.4 X  
4,874,639 10/1989 Matsui et al. ..... 427/240  
4,919,977 4/1990 Yamane et al. ..... 427/379

## FOREIGN PATENT DOCUMENTS

2228 3/1976 Japan  
30581 2/1982 Japan

Primary Examiner—Michael Lusignan  
Attorney, Agent, or Firm—Wegner, Cantor, Mueller & Player

## [57] ABSTRACT

A coating method contains a coating step for spraying the surface of a coating substrate paint with a paint and a drying step for drying the paint coated thereon. The paint coated on the substrate is then caused to flow or sag artificially within the coat in the drying step by application of an action from the outside at least in one of the coating and drying steps, namely, by heating or vibrating the paint coated thereon. During the flowing or sagging of the paint artificially, the substrate is rotated about its axis extending substantially horizontally in a longitudinal direction of the substrate at a speed which is high enough to rotate the substrate before the paint coated thereon substantially sag due to gravity yet which is low enough so as to cause no sagging as a result of centrifugal force.

28 Claims, 20 Drawing Sheets



FIG. 1





**FIG. 3****FIG. 4**

**FIG. 5****FIG. 6**

卷之三



៩  
១៩  
៤



**FIG.10****FIG.14****FIG.11****FIG.13****FIG.15****FIG.12**

**FIG.16**

**FIG. 17****FIG. 18**

**FIG.19**

**FIG. 20**

**FIG.21**

**FIG.22**



**FIG. 23**



**FIG. 24****FIG. 25**

**FIG. 29(a)****FIG. 29(b)**

**FIG. 26**

**FIG. 27(a)****FIG. 27 (b)**

**FIG. 27(c)****FIG. 27(d)**

**FIG. 27 (e)****FIG. 27 (f)**

**FIG. 28(a)****FIG. 28 (b)****FIG. 28 (c)**

**FIG. 28(d)****FIG. 28(e)**

## COATING METHOD

## BACKGROUND OF THE INVENTION

## 1. Field of the Invention

The present invention relates to a coating method and, more particularly, to a coating method in which a paint coated on a coating substrate is caused to flow or sag artificially by an outside action while rotating the substrate about its horizontal axis at least in one of a step of coating the substrate with the paint and a step of drying the paint coated on the substrate.

## 2. Description of Related Art

The subject matter of this application is related to the subject matter of commonly-assigned and copending application Ser. No. 07/100,767, now U.S. Pat. No. 4,874,639, of application Ser. No. 07/153,669, now abandoned, and of application Ser. No. 07/323,237, now U.S. Pat. No. 4,919,977.

Technology relating to the rotation of a coating substrate after coating is disclosed in Japanese Utility Model Publication (kokoku) No. 2,228/1976, Japanese Patent Publication (kokai) Nos. 30,581/1982 and 67,332/1973 as well as U.S. Pat. No. 4,092,953.

Other technology relating to coating a coating substrate is disclosed in Japanese Utility Model Publication (kokai) Nos. 80,930/1983, 109,430/1984, and 21,361/1975, Japanese Utility Model Publication (kokoku) No. 20,053/1981, Japanese Patent Publication (kokai) No. 4,471/1984, as well as U.S. Pat. Nos. 1,948,091, 2,658,008, and 2,598,163.

A coating method for coating an outer surface of a coating substrate such as a vehicle body generally includes a preparation step for preparing for the coating substrate to be coated with a part by removing dust from the substrate, a coating step for coating the coating substrate with the paint, and a drying step for drying the paint coated thereon. The drying step generally comprises setting and baking steps particularly when a thermosetting paint is used. The setting step is usually carried out prior to the baking step at a temperature which is lower than the ambient temperature during the baking step, for example, at room temperature or at the temperature ranging from 40° C. to 60° C. in order to volatilize a solvent slowly so as to cause no pinholes on the coating surface during the baking step which is usually carried out at approximately 140° C.

The coating substrate is held at a given position on a conveyance means such as a carriage while being conveyed during the preparation, coating, and drying steps.

A degree of flatness or smoothness on the surface of a coating on the coating substrate is one of standards for evaluating a quality of the coat surface. The higher a degree of flatness the smaller a degree of irregularities on a coating surface, thus producing a better coating surface. It is well known that a thicker film thickness of a paint may give a higher degree of flatness on a coating surface. A paint sprayed on the surface of a coating may be said to sag if it is visually observed that the paint coated thereon flows and finds traces on the coating surfaces by 1 mm to 2 mm until it is cured in the drying step. It may be defined herein that sags of the paint occur if such traces exceed at least 2 mm when visually observed. In other words, a sagging limit thickness of a coating is a film thickness beyond the maximum film thickness in which the coating does not sag and the coating in its sagging limit thickness is caused to sag at least in the drying step if it is left as it is after spraying.

On the contrary, a film thickness of the paint within its sagging limit thickness is a film thickness in which it does not sag in the drying step even if it is left as it was sprayed.

It is known that sags or drips of a paint coated on the substrate during the coating step are detrimental to the quality of the coating surface. Such sags or drips are caused when the paint coated thereon flow downwardly due to gravity. They become more likely to occur if the paint is coated in a film thickness which becomes thicker in one coating.

And it is a matter of course that the sags are caused more likely on a coated surface extending in an up-and-downward direction than on a coated surface extending in a horizontal direction. This enables the paint to be coated on the surface extending horizontally in a film thickness which is thicker than on the surface extending in an up-and-downward direction because the sags or drips of the paint little affect adversely the coating surface extending in a horizontal direction. If the film thickness of a coat on the horizontally extending surface is the same as that on the surface extending in an up-and-downward direction, the former can produce a degree of flatness which is higher than the latter because the paint coated on the horizontally extending surface of a coating surface becomes flattened due to a natural flow in the paint to an extent to which no sags substantially occur.

Conventionally, in order to provide a coat with a higher degree of flatness while preventing sags or drips of a paint coated on the surface of a coating substrate, there have been used paints which are lower in viscosity and less flowable. Even if such thermosetting paints are used, however, a sagging limit of the paint coated on the surface extending in an up-and-downward direction is as high as approximately 40  $\mu\text{m}$ . This sagging limit thickness, referred to sometimes as a sagging threshold value, is the maximum film thickness in which the paint does not substantially sag on the surface of a coating substrate extending in an up-and-downward direction.

Sags of the paint are likely to occur at initial stages of the setting and baking steps, particularly at the initial stage of the baking step so that a film thickness of a coat is determined by a film thickness of the paint coated on the surface of a coating substrate to such an extent that the paint does not sag on an up-and-downwardly extending surface thereof. Accordingly, in order to provide a coating in a film thickness larger than a sagging limit thickness of the paint, the coating step is repeated twice or more in the conventional coating method.

It is effective to rotate a coating substrate about its horizontal axis extending in a substantially horizontal direction of the substrate in order to provide a coating with a higher degree of flatness. In other words, even if the film thicknesses are the same, a coating with a higher degree of flatness may be given by utilizing a flowability of the paint in such a manner that a direction in which gravity acts upon a surface of the coating is artificially changed by rotating the substrate. This technology may produce a similar effect even if the paint is coated in a film thickness which is thicker than a sagging limit thickness of the paint to the contrary of conventional coating techniques.

## SUMMARY OF THE INVENTION

Therefore, the present invention has the object to provide a coating method that produces a coat with a

larger film thickness and with a higher degree of flatness on the surface of a coat than the surface of a coat which is obtained by the conventional method.

In order to achieve the object, the present invention involves altering a direction of the surface of a coating substrate in which gravity acts and utilizing a flowability of a paint coated on the surface thereof.

Thus the present invention consists of a coating method comprising: a coating step for spraying a surface of a coating substrate with a paint; and a drying step for drying the paint sprayed on the surface thereof; at least in one of the coating and drying steps an action is applied from outside so as to cause the paint coated thereon to flow or sag, while the substrate is rotated about its axis extending substantially horizontally in a longitudinal direction of the body at a speed which is high enough to rotate the body before the paint coated thereon substantially sags due to gravity yet which is low enough so as to cause no sagging as a result of centrifugal force.

In accordance with the present invention, the paint coated on the surface of the coating substrate is dried without sags or drips on the coat surface due to alteration of a direction of the coat surface in which gravity acts by rotating the coating substrate about its horizontal axis extending substantially horizontally in a longitudinal direction of the substrate.

The coating method according to the present invention permits a provision of a coat in a film thickness and with a degree of flatness by one coating, which is thicker and higher than that obtainable by the conventional coating method, respectively.

Furthermore, even if a film thickness of a coat coated on the coating substrate by the coating method according to the present invention is the same as that obtainable by the conventional method, the present invention provides the coat surface with a higher degree of flatness than that obtained by the latter.

If a coat surface has substantially the same degree of flatness as that obtainable by the conventional coating method, the coating method according to the present invention requires a film thickness thinner than that required by the conventional coating method, thus saving a quantity of the paint which is otherwise required to be consumed to a much greater extent.

The coating method according to the present invention is applicable to those paints used for the conventional coating method. Even if the paint is too flowable to be coated in a desired thin film thickness without sags or drips, it may be applied to the coating method according to the present invention if an ingredient such as a hybridizing agent which is added to increase its sagging threshold value would be reduced or removed from the conventional paint.

The coating method according to the present invention involves producing sags in an artificial manner from the outside at least in the coating or drying step. For this reason, even a paint that does not sag without actions from the outside may be used for the coating method according to the present invention. This enables a highly viscous paint to flow to such an extent to which the paint sags. This offers the great advantage that the paint coated in a film thickness which is thin enough to cause no sags in a usual state in the drying step can be caused to flow or sag during the drying step, as needed, thus making the paint coated thereon flowable and improving a degree of flatness on the coat surface. This coating method further presents the advantage that the

time required for an interval, for instance, between the first coating and the second coating can be saved when the coating step is desired to be repeatedly carried out plurally. Furthermore, attention is little required to be paid to an ingredient of the paint. A combination of the rotation of the substrate with a flowability of the paint created during at least one of the coating and drying steps can improve a degree of flatness on the coat surface even if the paint is coated in a thin film thickness.

10 The outside action that may cause the paint coated on the surface of the coating substrate to flow or sag in an artificial manner may include heating or a vibration. In usual cases, a thermosetting paint is heated in the setting step at room temperature or at a temperature that is lower than that in the baking step. In the coating method according to the present invention, however, the setting step can be carried out at a temperature as high as the baking step. By heating the coat on the substrate in the setting step at the temperature as high as in the baking step, the paint which usually has not flown or sagged in the setting and baking steps can be caused to flow or sag within the coat in the setting step, thus enabling the coat surface to become flattened and causing no pinholes on the coat surface.

15 While the coating substrate undergoes the outside action to allow the paint coated thereon to flow or sag within the coat in an artificial manner, it is rotated about its horizontal axis. An angle at which the substrate is coated thereabout is at least as great as 10 degree with respect to an angle at which the substrate is mounted. The substrate may be rotated about its horizontal axis continuously or intermittently in one direction or in alternate directions.

20 25 30 35 The coating substrate may be rotated at a speed which is high enough to rotate the substrate before the paint flows down or sags over an acceptable sagging limit thickness due to gravity yet which is low enough so as to cause no sagging as a result of centrifugal force.

40 Specifically, the acceptable sagging limit thickness is generally up to about 2 mm per minute, preferably up to 1 mm, when visually observed. If the paint is likely to flow down or sag at the rate exceeding the acceptable sagging limit, then the rotation of the substrate is reversed in the opposite direction. As a degree of flowing or sagging varies with the kind of a patient used, the maximum degree at which the paint does not flow or sag is determined experimentally in advance and the the speed of rotating the coating substrate is determined on the basis of the maximum degree of flowing or sagging obtained in advance experimentally.

45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 983

FIG. 7 is a side view showing the side portion of a vehicle-body conveying carriage for rotating the vehicle body.

FIG. 8 is a partially cut-out plane view showing the structure of a conveying means underneath a passageway on which the carriage travels.

FIG. 9 is a cross-sectional view taken along line X9—X9 of FIG. 8.

FIG. 10 is a cross-sectional side view showing a connecting portion at which the carriage is connected to a rotary jig.

FIG. 11 is a cross-sectional view taken along line X11—X11 of FIG. 10.

FIG. 12 is a plane view of FIG. 10.

FIG. 13 is a cross-sectional view taken along line X13—X13 of FIG. 10.

FIG. 14 is a cross-sectional view taken along line X14—X14 of FIG. 10.

FIG. 15 is a plane view of FIG. 14.

FIG. 16 is a graph showing the relationship of the setting and baking times vs. speeds at which the paint sags.

FIG. 17 is a view showing a preferred example of an oven for drying the paint coated on the vehicle body.

FIG. 18 is a view showing a combination of the oven of FIG. 17 with a system.

FIG. 19 is a view showing a preferred manner in which the vehicle body is dried.

FIG. 20 is a side view showing a carriage with the vehicle body mounted thereon and a passageway on which the carriage travels.

FIG. 21 is a cross-sectional view showing the detail of the portion indicated by reference symbol VI in FIG. 20.

FIG. 22 is an enlarged view showing the essential portion of a second example according to the present invention.

FIG. 23 is a side view showing a third example according to the present invention.

FIGS. 24 and 25 are each a graph showing the relationship of times vs. speeds with respect to a fourth example according to the present invention.

FIG. 26 is a graph showing the relationship of the number of revolutions vs. film thicknesses of coatings.

FIGS. 27(a) to 27(f) are each a graph showing speeds of paint sagging during the setting and baking steps without rotation of the substrate coated with a thermosetting paint in varying film thicknesses.

FIGS. 28(a) to 28(e) are each a graph showing speeds of paint sagging during the setting and baking steps without rotation of the substrate coated with a two-liquid type urethane paint in varying film thicknesses.

FIG. 29(a) and 29(b) are each a graph showing speeds of paint sagging during the baking step without rotation of the substrate coated with a powder paint in varying film thicknesses.

#### DETAILED DESCRIPTION OF THE PREFERRED EMBODIMENTS

##### Outline of Coating Method

FIG. 1 shows an outline of the whole steps of the coating method according to the present invention, in which a vehicle body W as a coating substrate is coated with a paint. As shown in FIG. 1, the coating method according to the present invention comprises roughly the preparation step P1, the coating step P2, the setting step P3, and the baking step P4. In this specification, the terms "drying step" is intended to mean a

sequential combination of the setting step P3 with the baking step P4, unless otherwise stated specifically.

The vehicle body W is first undercoated by conventional methods such as electrodeposition. The vehicle body W undercoated is conveyed on a carriage D to the preparation step P1. In the preparation step P1, dust and other foreign materials are removed from the inside and the outside of the vehicle body W, for example, by vacuum suction or air blowing for subsequent coating procedures. Then the vehicle body W is intercoated in conventional manner in the coating step P2 and the intercoated paint is cured in the setting step P3 and baked in the baking step P4. The body W so intercoated is then overcoated again in the coating step P2. Thereafter, the body W overcoated is cured in the setting step P3 and baked in the baking step P4. The overcoated vehicle body W is then conveyed to an assembly line.

##### Removal of Dust

In the preparation step P1, dust and other foreign materials are removed from the inside and outside of the vehicle body W by vacuum suction or air blowing. In the preparation step P1, the body W may be preferably rotated about its horizontal axis I, i.e., about an axis extending substantially horizontally in a longitudinal direction of the body W, as will be described in detail in conjunction with FIG. 2.

The rotation of the body W may readily remove dust and other foreign materials from corner portions inside a roof panel, a side sill and other partially closed sections which would not otherwise be removed without rotation of the body W.

##### Paints

The paints to be used for the coating method according to the present invention may be any paint which has been conventionally used for coating a coating substrate and may include, for example, thermosetting paints, two-component type paints, powder paints and so on. The paints may be conveniently chosen depending upon the kind of coating processes and the outside action to be applied as well as the speed of rotation. As needed, the paints may be used, for example, by adding a sags-preventing agent thereto or by diluting them with a solvent on site.

Particularly, paints to be used for coating the vehicle body W for an automobile may be ones having a number mean molecular weight ranging from about 2,000 to about 20,000 and include a solid coat of conventional type and of high solid type, a metallic base coat of conventional type and of high solid type, and a metallic clear coat of conventional type and of high solid type. The solid coat of an alkyd melamine resin of conventional type may have a number mean molecular weight ranging from about 4,000 to about 5,000 and of high solid type from about 2,000 to 3,000; the metallic base coat of an acrylic melamine resin of conventional type may have a number mean molecular weight from about 15,000 to about 20,000 and of high solid type from about 2,000 to about 3,000; the metallic clear coat of an acrylic melamine resin of conventional type may have a number mean molecular weight from about 5,000 to about 6,000 and of high solid type from about 2,000 to about 3,000; and the solid coat of a urethane isocyanate resin of conventional type may have a number mean molecular weight from about 7,000 to about 10,000 and of high solid type from about 2,000 to about 3,000. The paints

having a number mean molecular weight below about 2,000, on the one hand, are in many cases of the type in which they are cured by electron beams or by ultraviolet rays and they are hard and frail, when cured, leading to the shortening of durability, because their density of cross-linkage is too high. Thus such paints are inappropriate for coating exterior panels of the vehicle body. The paints having a number mean molecular weight above 20,000 on the other, are of the type in which they have a very high viscosity so that they require a large amount of a solvent to dilute. Thus high costs are required to treat the solvent discharged. A latex polymer with a number mean molecular weight over 200,000 is not appropriate because its viscosity is elevated immediately after spraying, thus adversely affecting a degree of flatness on a coating surface.

#### Coating of The Paint

In the coating step P2, the paint may be sprayed on a surface of the coating substrate in a desired film thickness which is thinner or thicker than a sagging threshold value of a paint to be coated on the surface thereof.

If the conventional paint is used, it may be coated on the surface of the body W by spraying in a film thickness as thick as, for example, 35  $\mu\text{m}$ , which is thinner than its sagging threshold value of about 40  $\mu\text{m}$ , as have been described hereinabove. In this case, no sags or drips are caused and the paint little flows due to gravity, whereby the rotation of the body W is not necessarily required for the purpose of preventing sags only. In order to provide a coat surface with a higher degree of flatness, however, the paint coated thereon may be preferably rotated in a manner as will be described hereinafter.

The paint may be coated on the surface of the substrate by spraying in a film thickness as thick as, for example, 65  $\mu\text{m}$ , which is thicker than its sagging threshold value. In this case, in order to prevent the paint from sagging, the substrate is rotated about its horizontal axis in a manner as will be described hereinbelow.

#### Drying of The Paint Coated

As have been described hereinabove, the drying step comprises sequential setting and baking steps P3 and P4.

##### a. Setting Step P3:

The vehicle body W coated with the paint in the coating step P2 is then conveyed on the carriage to the initial stage of the drying step, namely, to the setting step P3, where it is cured to a partial extent at a temperature ranging from 20° C. to 60° C. by slowly volatilizing a volatilizable solvent to form a highly surface coating for the body without pinholes.

If the paint is coated on the body W in the coating step P2 in a film thickness thin enough to cause no sagging due to gravity yet to sag in an artificial manner by an action to be applied from the outside (hereinafter referred to sometimes as "outside action") in a manner as will be described hereinafter, the body W may be heated in the setting step P3 at a temperature which is substantially as high as the temperature during the baking step P4, for example along the line indicated by the dot-dash line  $\alpha$  as shown in FIG. 16. The heating in the setting step P3 at such higher temperatures enables the paint coated thereon to flow in the coated paint causing sags even if the paint could not sag when coated in the film thickness below its sagging threshold value.

If the paint coated thereon in the coating step P2 is in a film thickness which is thicker than its sagging threshold value, the paint coated may be partially cured in an initial stage of the setting step P3 and then subjected to application of the outside action to cause sagging during the setting step P3.

While the vehicle body W is treated by application of the outside action, the body W is rotated about its horizontal axis  $l$  in a manner as shown in FIG. 2 and as will be described more in detail.

##### b. Baking Step P4:

The vehicle body W set in the setting step P3 is then conveyed by the carriage to the baking step P4 where it is continued to be heated at substantially the same temperature as that at the final stage of the setting step P3 or where the temperature is elevated to baking temperatures, for example, along the dot-dash line indicated by  $\beta$  in FIG. 16.

If the paint coated on the substrate is still flowable to an extent that it sags by means of application of the outside action when the body W is conveyed to the baking step P4 from the setting step P3, the rotation of the coating substrate may be preferably carried out during the baking step P4 while the outside action is applied thereto.

If the coating on the surface of the substrate is cured to a sufficient extent during the setting step P3 and if the paint coated thereon does not substantially flow or sag, the rotation of the body W is not necessarily required. For the purpose of heating the coat surface uniformly, however, the body W may be rotated in a manner as will be described hereinafter.

#### Outside Action

The action to be applied from the outside at least in one of the coating step and the drying step may be any means that exercises an effect or influence upon an inner movement of a paint coated on the surface of a substrate in a direction in which the paint substantially flows or sags. Application of the outside action permits a provision of flowability of the paint coated thereon to such an extent that it sags even if the paint does not flow due to gravity. The action to be applied from the outside may include, for example, heating from various heating sources and a vibration such as a mechanical vibration or an acoustic vibration. In accordance with the present invention, the rotation of the substrate is carried out during application of the outside action thereto.

#### Rotation of the Coating Substrate

Referring to FIG. 2, FIG. 2(a) shows an original position at which the body W is mounted on the carriage. FIG. 2(b) shows a position of the body W in which it is rotated at 45 degrees from the original position of FIG. 2(a). FIGS. 2(c), (d), and (e) show positions at which it is rotated at 90 degrees, 135 degrees, and 180 degrees, respectively, from the original position thereof. As shown in FIGS. 2(f), (g), and (h), the body W is further rotated at 225 degrees, 270 degrees, and 315 degrees, respectively, from the original position shown in FIG. 2(a). FIG. 2(i) shows the position at which the body is rotated at 360 degrees from and returned to the original position of FIG. 2(a). It should be understood that FIG. 2 is shown merely as references and that the body W may take any position.

The rotation of the body W may be carried out on the carriage continuously or intermittently in one direction

or in alternate directions in a cycle of rotation in which the body W is turned about its horizontal axis so as to allow every vertically cross-sectional portion of the body W passing through the center of its horizontal axis to pass equal occasions through the direction of gravity passing through the center thereof. If the body W is rotated in one direction, the rotation may be continuously or intermittently carried out in a clockwise direction in FIG. 2, for example, in a cycle from the original position of FIG. 2(a) through FIGS. 2(b), (c), (d), (e), (f), (g), and (h) to the original position of FIG. 2(i). If it is rotated continuously or intermittently in alternate directions, the rotation may be carried out first in the clockwise direction in FIG. 2, for example, in a first quarter of one cycle from the original position of FIG. 2(a) through FIG. 2(b) to the position of FIG. 2(c) and then reversed back in a counterclockwise direction in a second quarter thereof from FIG. 2(c) through FIG. 2(b) to the original position of FIG. 2(a) and then in a third and quarter thereof from the original position of FIG. 2(i), i.e., FIG. 2(a), through FIG. 2(h) to the position of FIG. 2(g). In this case, the rotation of the body W is reversed again in a counterclockwise direction in a fourth quarter of one cycle from the position of FIG. 2(g) through FIG. 2(h) to the original position of FIG. 2(i), namely, FIG. 2(a). Furthermore, for example, if the rotation of the body W is reversed at the angle of 135 degrees, the body W is rotated first in a clockwise direction from the original position of FIG. 2(a) through FIGS. 2(b) and 2(c) to FIG. 2(d), and the rotation is reversed back in a counter-clockwise direction therefrom through FIGS. 2(c) and (b) to FIG. 2(a). The body W is continued to be rotated therefrom, namely, from FIG. 2(i) through FIGS. 2(h), (g) to FIG. 2(f) and then reversed again in a clockwise direction therefrom through FIGS. 2(g) and (h) to FIG. 2(i), namely, to the original position of FIG. 2(a). It is to be noted that the rotation of the body W may be reversed at any angle and it is not restricted at any means to those as have been described hereinabove.

As an angle at which the body W is rotated about its horizontal axis depends upon a degree to which the paint coated on the body W is flowable, it is to be noted that the rotation of the body W should be carried out at angles at which the paint coated thereon does not exceed its sagging limit, as will be described more in detail. If the paint would be likely to exceed its sagging limit while the body W is rotated in one direction, then the rotation of the body W should be reversed in the opposite direction to prevent the paint from dropping.

A speed of rotation of the body W is a speed which is high enough to rotate the body from a vertical position to a horizontal position before the paint coated thereon substantially sags due to gravity by allowing the gravity applied to the paint coated thereon to outweigh a viscosity of the paint as a result of application of the outside action rendering the paint flowable, yet which is low enough so as to cause no sagging as a result of centrifugal force. The maximum value for the speed of rotation is restricted to a range of speeds of rotation within which no sags are caused as a result of centrifugal force caused by the rotation of the body W on a coat of the paint a flowability of which becomes higher by application of the outside action. It is noted herein that the speed of rotation is determined on the basis of the maximum speed of paint sagging which in turn is preferably determined experimentally in advance. The relationship of the speed of rotation with a film thickness

will be described in detail hereinbelow in conjunction with FIG. 26, and some discussion will be made therein on determination of the maximum speed of rotation vs. the film thicknesses of the paint.

#### Relationship of Film Thickness of Paint with Speed of Rotation

For the coating method according to the present invention, the maximum and minimum numbers of revolution of the vehicle body W may be determined per a film thickness of a paint to be coated on a surface of the body W. The maximum number of revolutions of the body W may be defined as the maximum value at which the paint coated is caused to sag as a result of centrifugal force, i.e., at the maximum value at which sags are caused as a result thereof, while the minimum number of revolutions of the body W may be defined as the minimum value at which the paint coated is not caused to sag, i.e., as the minimum value at which sags are prevented. The maximum value of revolutions thereof is reduced as a film thickness of the paint becomes thicker, while the minimum value thereof rises as a film thickness thereof becomes thicker. And the maximum film thickness of the paint may be defined as a value at which the maximum number of rotations coincides with the minimum number thereof.

Referring now to FIG. 26, the dashed line E is shown to denote the maximum number of revolutions thereof and the solid line F is shown to denote the minimum number of revolutions thereof. The tests are carried out in the same conditions as in the tests done in accordance with the conditions as shown in FIGS. 3 and 4, provided that the test results are obtained when the test pieces were rotated in a rotational distance of 30 cm. It is to be noted that the relationship of the number of rotations with the distance may vary with the change of the distance because the speed of rotation at the tip of the substrate changes.

It has now been found from the test results as shown in FIG. 26 that the maximum film thickness of the paint so defined hereinabove is approximately 185  $\mu\text{m}$ .

#### Relationship of Film Thickness of Paint with Speed of Paint Sagging

FIG. 3 demonstrates the influence of film thicknesses of a paint upon the speed at which the paint sags. The speeds of paint sagging are measured for three different film thicknesses of 40  $\mu\text{m}$ , 53  $\mu\text{m}$ , and 65  $\mu\text{m}$ . As shown in FIG. 3, it has been found that a peak of the sagging speed appears at initial stages of the setting and baking steps in each case.

#### Relationship of Film Thickness with Degree of flatness

FIG. 4 shows the influence of the rotation of the vehicle body W about its horizontal axis upon degrees of flatness on the coat surface of the coating substrate expressed in a degree of image gross.

In FIG. 4, reference symbol A denotes a state of the coat surface obtained without the rotation of the vehicle body W in conventional manner. Reference symbol B denotes a state of the coat surface obtained by the rotation of the body W which is carried out in a clockwise direction at an angle of 90 degree, namely, from the position of FIG. 2(a) through FIG. 2(b) to FIG. 2(c) and then reversed in the opposite direction back to the original position of FIG. 2(a) from which, namely, from FIG. 2(i), the body W in turn is continued to be rotated in the same direction through FIG. 2(h) to FIG. 2(g).

and then turned again in the counterclockwise direction therefrom through FIG. 2(h) to the original position of FIG. 2(i). Reference symbol C demonstrates a state of the coat obtained when the rotation of the body W is carried out first in a clockwise direction at the angle of 135 degrees, namely, from the original position of FIG. 2(a) through FIGS. 2(b) and (c) to FIG. 2(d) and reversed in a counterclockwise direction therefrom through FIGS. 2(c), (b) to FIG. 2(a) from which, namely, from FIG. 2(i), the rotation is continued to FIG. 2(h) and then reversed again in a clockwise direction to the original position of FIG. 2. Reference symbol D demonstrates a state of the surface of the coat which was obtained by the rotation of the body W at the angle of 180 degrees in a clockwise direction from the position of FIGS. 2(a) to (e) and then by reversal of the rotation in a counterclockwise direction back to the original position of FIG. 2(a). In FIG. 4, reference symbol E shows a state of the coat surface obtained when the body W is continuously rotated around in one way from the original position of FIG. 2(a) through FIGS. 2(b), (c), (d), (e), (f), (g), and (h) to the original position of FIG. 2(i), namely, FIG. 2(a).

As shown in FIG. 4, it is found that higher degrees of flatness on the coat surfaces are given when the body W is rotated as in the cases of reference symbols B, C, D and E, than reference symbol A, if the film thicknesses are the same. It is also found that a higher degree of flatness can be produced when the body W is rotated continuously in one direction at the angle of 360 degrees than when the rotation is carried out in one direction and then reversed in the opposite direction or directions. It is further found in the result shown in FIG. 4 that the coat obtainable without rotation of the body W is thin in a film thickness, thus leading to a lower degree of flatness and producing a limit upon thickening its film thickness.

When the film thickness of 65  $\mu\text{m}$  was formed on the body W by rotating continuously in one direction at the angle of 360 degrees, a degree of flatness is "87" when expressed in an image gloss (I.G.) as a degree of image, namely, the lowest limit value when the PGD value is 1.0. In the case of the coat in the film thickness of 40  $\mu\text{m}$  formed without rotation, a degree of flatness is "58" when expressed in the image gloss (I.G.), or the lowest limit value when the PGD value is 0.7, while the coat in the film thickness of 40  $\mu\text{m}$  formed by the continuous rotation in one direction at the angle of 360 degrees provides a degree of flatness which is "68" when expressed in the image gloss (I.G.) as a degree of image sharpness, or the lowest limit value when the PGD degree is 0.8. It is understood that the definition for the image gloss (I.G.) in the image sharpness degree is a percentage of an image sharpness on an objective coat surface on the basis of the image gloss of "100" when a mirror surface of a black glass is used, and a PGD value is a value rating identification degrees of reflected images from 1.0. The PGD value gets lower as the degree of flatness gets lower.

The data shown in FIGS. 3 and 4 were obtained by 60 overcoating in the coating step P2 above under following test conditions:

- (a) Paint: melamine alkid (black)
- Viscosity: 22 seconds/20° C. (measured by Ford Cup #4)
- (b) Film coater: Minibell (16,000 r.p.m.)
- Shaping air: 2.0 kg./cm<sup>2</sup> c)
- (c) Spraying amounts: sprayed two times

First time: 100 cc/minute  
 Second time: 150-200 cc/minute  
 (d) Setting time/temperature: 10 minutes/room temperature  
 (e) Baking temperature/time: 140° C./25 minutes  
 (f) Degree of flatness on overcoat surface: 0.6 (PGD) (intercoat on PE tape)  
 (g) Time period for rotation and reversal: 10 minutes (for the setting step) 10 minutes (for the baking step)  
 (h) Coating Substrate: The side surfaces of a square pipe with a 30 cm side are coated and supported rotatably at its center.  
 (i) Rotational speeds: 6, 30, and 60 r.p.m.  
 It is found that there is no variation in degrees of flatness on the coat surfaces obtained by the different speeds of rotation.

#### Oven

The paint coated on the surface of the coating substrate such as the vehicle body is heated in an oven as shown in FIGS. 17 and 18 in the setting step P3—when it is heated at the temperature as high as that during the baking step P4—and in the baking step P4.

As shown in FIG. 17, the oven 60 may be designed to cover right-hand and left-hand sides and a top side of the vehicle body W with a housing consisting of a number of infrared panels 61. As shown in FIG. 18, it may also be designed to use a housing consisting of high-frequency induction coils 62 in place of the infrared panels used for the oven in FIG. 17. In both cases, it is preferred to heat the top side of the body W at sufficiently elevated temperatures in order to prevent a convection of air within the oven and to avoid occurrence of floating dust as much as possible. As shown in FIG. 18, the oven is designed to apply electricity to the coils 62 through a rectifier 66 and an inverter 67, and to control a magnetic field constant by regulating the inverter 67 by a control unit 68. The oven of the type as shown in FIG. 18 is preferably employed in order to heat the body W in a uniform manner because the magnetic field can be held constant in correspondence with a change in a clearance between the body W and the coils 62 attendant upon the rotation of the body W.

FIG. 19 shows an example of a heating system in which the vehicle body W is heated from the inside. Together with this heating system, the oven of the type as shown in FIGS. 17 and 18 or any other oven of the type used conventionally may be employed. The heating system as shown in FIG. 19 is such that a hollow cylinder member 71 with a number of small holes is detachably mounted within the body W by connecting its both ends to a pair of front and rear rotation jigs 1F and 1R, respectively, disposed on the carriage. Warm air is blown in the hollow cylinder member 71 through a hose 72 connected through a rotary joint (not shown) to the cylinder member 71 and further into the inside of the body W through the holes provided on the cylinder member 71. With this arrangement, the body W may be heated from the inside in addition to from the outside.

#### Rotation Jig

The vehicle body W is mounted horizontally on the carriage through a pair of rotation jigs so as to be rotatable about its axis extending horizontally in a longitudinal direction of the body W.

FIG. 5 shows a front rotation jig 1F for horizontally supporting a forward portion of the body W. The front rotation jig 1F comprises a pair of left-hand and right-

hand mounting brackets 2, a pair of left-hand and right-hand stays 3 welded to the corresponding left-hand and right-hand mounting brackets 2 and a connection bar 4 for connecting the pair of the stays 3, and a rotary shaft 5 connected integrally to the connection bar 4. The front rotation jig 1F is fixed at its portions of the brackets 2 to a forward end portion of a front reinforcing member of the vehicle body W such as a front side frame 11. To the front side frame 11 is usually welded mounting brackets 12 for mounting a bumper (not shown), and the brackets 2 are fixed with bolts (not shown) to the brackets 12 on the side of the body W.

FIG. 6 shows a rear rotation jig 1R for horizontally supporting a rearward portion of the vehicle body W, which substantially the same structure as the front rotation jig 1F. In the drawing, the same elements for the rear rotation jig 1R as for the front rotation jig 1F are provided with the same reference numerals as the latter. The mounting of the rear rotation jig 1R to the vehicle body W is effected by fixing brackets 2 with bolts (not shown) to the floor frame 13 disposed at a rearward end portion of the vehicle body W as a rigidity adding member. Alternatively, the rear rotation jig 1R may be mounted to the body W through a bracket for mounting the bumper, the bracket being welded to a rearward end portion of the floor frame 13.

The front and rear rotation jigs 1F and 1R are mounted to the body W in such a manner that their respective rotary shafts 5 extend horizontally on the same straight line in its longitudinal direction when the body W is mounted on the carriage D through the front and rear rotation jigs 1F and 1R. The very straight line is the horizontal axis 1 about which the body W is rotated. It is preferred that the horizontal axis is designed so as to pass through the center of gravity G of the body W as shown in FIG. 7. The arrangement for the horizontal axis 1 to pass through the center of gravity G serves as preventing a large deviation of a speed of rotation. This can prevent an impact upon the body W accompanied with the large deviation in rotation, thus preventing the paint coated from sagging.

The front and rear rotation jigs 1F and 1R may be prepared for exclusive use with the kind of vehicle bodies.

#### Carriage

The carriage which will be described hereinbelow is a carriage that may be used at least during the coating step P2 and/or in the setting step P3 and that is provided with a mechanism for rotating or turning the vehicle body W about its horizontal axis 1 extending in a longitudinal direction thereof.

Referring to FIG. 7, the carriage D is shown to include a base 21 and wheels 22 mounted to the base 21 with the wheels 22 arranged to operatively run on rails 23. On the base 21 is mounted one front support 24, two intermediate supports 25 and 26, and one rear support 27, each standing upright from the base 21, as shown in the order from the forward side to the rearward side in a direction in which the vehicle body W is conveyed. Between the intermediate supports 25, 26 and the rear support 27 is formed a space 28 within which the body W is mounted through the front and rear rotation jigs 1F and 1R.

The vehicle body W is loaded in the space 28 and supported rotatably at its forward portion by the intermediate support 26 through the front rotation jig 1F and

at its rearward portion by the rear support 27 through the rear rotation jig 1R.

As shown in FIGS. 10, 11, and 12, on the one hand, the intermediate support 26 is provided at its top surface with a groove 26a which in turn is designed so as to engage or disengage the rotary shift 5 of the front rotation jig 1F with or from the support 26 in a downward direction or in an upward direction.

As shown in FIGS. 10, 14, and 15, on the other hand, the rear support 27 is provided at its top surface with a groove 27a which engages or disengages the rotary shaft 5 of the rear rotation jig 1R with or from the rear support 27. The rear rotation jig 1R is further provided with a groove 27b in a shape corresponding to a flange portion 5a provided on the rotary shaft 5 of the rear rotation jig 1R, the groove being communicated with the groove 27a.

This arrangement permits the engagement or disengagement of the rotary shifts 5 with or from the front and rear rotation jigs 1F and 1R in a downward direction or in an upward direction, but it allows the rear rotation jig 1R to be unmovable in a longitudinal direction in which the horizontal axis extends due to a stopper action of the flange portion 5a.

As shown in FIGS. 10, 11, and 12, the rotary shaft 5 of the front rotation jig 1F is provided at its end portion with a connection portion 5b through which a force of rotation of the rotary shaft 5 of the front rotation jig 1F is applied to the vehicle body W, as will be described hereinbelow.

From the base 21 extends downwardly a stay 29 to a lower end portion of which is connected a retraction wire 30. The retraction wire 30 is of endless type and is drivable in one direction by a motor (not shown). The retraction wire 30 thus drives the carriage D in a predetermined direction in which the body W should be conveyed. The motor should be disposed in a safe place from the viewpoint of security from explosion.

The rotation of the vehicle body W may be carried out using a movement of the carriage D, that is, using a displacement of the carriage D with respect to the rails 23. The displacement of the carriage D may be converted to a force of rotation using a mechanism 31 for converting the displacement of the carriage D into rotation. The mechanism 31 comprises a rotary shaft 32 supported rotatably by the base 21 and extending in a vertical direction from the base 21, a sprocket 33 fixed on the lower end portion of the rotary shaft 32, and a chain 34 engaged with the sprocket 33. The chain 34 is disposed in parallel to the retraction wire 30 in such a state that it does not move along the rails 23. As the carriage D is retracted by the retraction wire 30, the sprocket 33 allows the rotary shaft 32 to rotate because the chain 34 is unmovable.

A force of rotation of the rotary shaft 32 is transmitted to the rotary shaft 5 of the front rotation jig 1F through a transmitting mechanism 35 which comprises a casing 36 fixed on a rearward side surface of the front support 24, a rotary shaft 37 supported rotatably to the casing 36 and extending in a longitudinal direction of the body W, a pair of bevel gears 38 and 39 for rotating the rotary shaft 37 in association with the rotary shaft 32, and a connection shaft 40 connected to the front support 25 rotatably and slidably in the longitudinal direction thereof. The connection shaft 40 is spline connected to the rotary shaft 37, as indicated by reference numeral 41 in FIG. 7. This construction permits a rotation of the connection shaft 32 to rotate the rotary shaft

40. It is understood that the rotary shaft 37 and the connection shaft 40 are arranged so as to be located on the horizontal axis 1 extending in a longitudinal direction of the body W. The connection shaft 40 is connected to or disconnected from the front rotary shaft 5 of the front rotation jig 1F. More specifically, as shown in FIGS. 10 to 12, the front rotary shaft 5 of the front rotation jig 1F is provided at its end portion with a connecting portion 5b in a cross shape, while the connection shaft 40 is provided at its end portion with a box member 40a having an engaging hollow portion 40c that is engageable tightly with the connection portion 5b of the front rotary shaft 5 as shown in FIGS. 10 and 12. By slidably moving the connection shaft 40 by a rod 43, for example, using a hydraulic cylinder 42, the connection portion 5b is connected to or disconnected from the box member 40a at its engaging hollow portion 40c. The connection shaft 40 is rotatable integrally with the rotary shaft 5. The rod 43 is disposed in a ring groove 40b formed on an outer periphery of the box member 40a, as shown in FIG. 10, in order to cause no interference with the rotation of the connection shaft 40. With the above arrangement, the front and rear rotary shafts 5 of the respective front and rear rotation jigs 1F and 1R are supported by the intermediate support 26 and the rear support 27 so as to be rotatable about the horizontal and longitudinal axis yet unmovable in a longitudinal direction of the body W, when the body W is lowered with respect to the carriage D in a state that the connection shaft 40 is displaced toward the right in FIG. 7. Thereafter, the connection portion 5b of the rotary shaft 5 is engaged with the connection shaft 40 through the engaging hollow portion 40c thereof, whereby the body W is allowed to rotate about the predetermined horizontal axis 1 by retracting the carriage D by means of the retraction wire 30. The vehicle body W can be unloaded from the carriage D in the order reverse to that described above.

Referring now to FIG. 20, there is shown another example of a combination of a carriage D' with rails on which the carriage D' travels. The carriage D' has substantially the same structure as the carriage D shown in FIG. 7 so that the same elements are provided with the same reference numerals and symbols and that a description on those elements are omitted for brevity of description.

In this example, the rails R are designed to be of a waveform shape curved upwardly and downwardly, as indicated by paint sagging, namely, a speed in which the paint sags, becomes high. Such an area may be the setting step P3 and an initial stage of the baking step P4. The other range of the rails R is straight. While the carriage D' travels a waveform range of the rails R1, it is swung substantially in upward and downward directions.

As shown in FIG. 21, a mechanism 35 for converting an upward-and-downward movement to rotation may be designed to comprise a rotary shaft 32 consisting of an upper rotary shaft portion 32a and a lower rotary shaft portion 32b, and the upper rotary shaft portion 32a is spline connected to the lower rotary shaft portion 32b. A spline-connectable portion 32c of the lower rotary shaft portion 32b is displaceable vertically, and a compression spring 32d is interposed between the spline-connectable portion 32c and the main body of the lower rotary shaft portion 32b, thus urging the spline-connectable portion 32c always in an upward direction. In the drawings, reference numeral 32e denotes a key.

The above arrangement for the combination of the carriage D' with the rails R permits the rotation of the body W about its horizontal axis 1 and a vibration of the carriage D' in an upward-and-downward movement, thus enabling the paint coated to be vibrated during the setting step P3 and/or during the initial stage of the baking step P4. The vibration of the carriage D' changes a direction in which gravity acts on the paint coated, thus altering the absolute value of a force acting upon the paint coated.

Turning now to FIG. 22, there is shown another example of a mechanism 35 for converting the upward-and-downward movement to rotation, in which the same elements are provided with the same reference numerals and symbols as the above embodiments. The mechanism 35 of this example is designed to use a backlash of a pair of first and second bevel gears 38 and 39, respectively, to apply a vibration to the paint coated on a surface of the vehicle body W. The mechanism 35 comprises a housing 36 which is provided with a pressure chamber 36a. A piston 36b is then inserted into the pressure chamber 36a and is fixed to a forward end surface of the first bevel gear 38 which in turn is mounted movably to the rotary shaft 5 of the front rotation jig 1F in a longitudinal direction of the body W. A spring 60 is mounted between a rearward inner side surface of the housing 36 and a rearward side surface of the first bevel gear 38, thus urging the first bevel gear 38 in a forward direction. Into the pressure chamber 36a is intermittently fed compressed air through an air inlet tube 62. In the drawing, reference numeral 38a denotes a key and 38c denotes a stopper.

As shown in FIG. 22, a force for driving rotation is produced by an engagement of the chain 34 with the sprocket 31 so that a back clash always occurs by the sprocket 31 and the chain 34. The above arrangement for the mechanism 35 amplifies the back clash.

Turning further to FIG. 23, there is shown a further example of a system in which a vibration is provided on the paint coated on a surface of the vehicle body W. This example shows a speaker 50 that produces an impulse sound transmitted to the coat surface through air, thus creating a vibration to cause the paint to flow or sag and forming a uniform film thickness of the coat with a higher degree of flatness.

FIGS. 24 and 25 show each a still further example in which speeds for conveying the carriage D are varied, as shown therein, by changing the retracting action by the retractable wire 30. The speed of rotating the vehicle body W may be varied, for example, by deviating the horizontal axis in an upward or downward direction from gravity of the body W. While the running speeds of the carriage D are varied, the body W is rotated in the manner as have been described hereinabove.

Those examples as have been described hereinabove may be combined with the other examples in an appropriate manner.

#### Variants

60 If an overcoating step is carried out after an intercoating step, a wet rubbing treatment can be cancelled which is otherwise done after the baking step for the intercoat.

65 The rotation of the vehicle body W may be carried out either in the intercoating step or in the overcoating step. A final quality of the overcoat depends primarily upon the intercoat so that the rotation of the body W during the intercoating step provides a higher quality of

the intercoat, thus cancelling the wet rubbing treatment. It is to be noted, however, that the rotation of the body W during the overcoating step can provide an overcoat surface in a higher quality even if no wet rubbing treatment would be made for the intercoat.

If the body W is rotated during the overcoating step and if an overcoating paint having a low sagging threshold value is coated in a thin film thickness, a paint with a color different from the overcoating paint may be used to see the color of the intercoat through the overcoat, thus providing a color different from the colors of the paints used.

Regardless of travel or suspension of the carriage D, the body W may be switched from a state of rotation of the carriage D to a state of suspension thereof or vice versa by an actuator for exclusive use, such as an air motor. A direction in which the body W is rotated may be changed by such an actuator. For example, as shown in FIG. 7, the sprocket 33 may be provided with first and second pairs of chains 34 engageable with each other from the opposite side in a radial direction, thus operatively driving each of the chains 34. With this arrangement, the rotation of the vehicle body W may be controlled according to the following operation modes: In a mode in which the first pair of chains 34 are suspended while the second pair of chains are released free, the vehicle body W is allowed to rotate in one direction as the carriage D runs. In a mode in which the first pair of chains and second chains are released free and the second pair of chains are suspended, the vehicle body W is allowed to rotate in the direction opposite to that in the mode as the carriage D runs. In a mode where both the first and second pairs of chains are released free, the vehicle body W are not allowed to rotate in association of the running of the carriage D. In a mode where the first pair of chains are driven in one direction and the second pair of chains are released free, the vehicle body W is allowed to rotate in one direction while the carriage D is suspended. In a mode in which the first pair of chains are driven in the other direction and the second pair of chains are released free (or the first pair of chains are released free and the second pair thereof are driven in the other direction), the vehicle body W is rotated in the direction opposite to in the mode even if the carriage D is suspended.

In the above cases, a rack bar may be likewise used in place of the chains. If the rack bars are disposed in a fixed state when the vehicle body W is rotated while the carriage D travels, they may be arranged in a constantly spaced relationship or in an arbitrarily spaced relationship on right-hand and left-hand rows, thus rotating the body W in an arbitrary direction and suspending the rotation of the body W at an arbitrary position.

The present invention will be described more in detail by way of examples.

## EXAMPLE 1

### a. Treatment of Coating Substrate

A cold rolled steel plate which has been usually used for vehicle bodies was subjected to the zinc phosphate treatment in conventional manner and the steel plate was then coated with an undercoating paint to cationic electrodeposition at 175° C. for 30 minutes, thus producing an undercoating with a film thickness of about 30  $\mu\text{m}$ . The undercoating was then sprayed with an oil-free polyester intercoating paint with a gray color

and baked at 140° C. for 25 minutes forming an intercoating with the film thickness of 35  $\mu\text{m}$ .

### b. Overcoating

As an overcoating paint, a paint of the type being dilutable with a solvent was sprayed on the intercoating in varying film thicknesses as shown in Table 1 below and treated under the following conditions:

#### (a) Paint

(1) Agent: melamine alkyd high solid thermosetting type (black, average molecular weight of main resin

(2) Viscosity for spraying: 20 seconds (measured by Ford Cup #4 at 20° C.)

(3) Involatilizables: 48% by weight

(4) Solvent: toluene, 25 parts by weight; Solvesso 100, 25 parts by weight; Solvesso 150, 50 parts by weight

(5) Agent for preventing sags: cross-linked acrylic resin powders, 3% by weight based on the unvolatilizables

(b) Film coater: Minibell (bell size: 60 mm; Lundsberg Japan, K.K.); sprayed once

Revolutions, 1,8000 r.p.m.

Shaping air: 3.0 kg./cm<sup>2</sup>

Voltage: 90 kv

Distance from gun: 30 cm

(c) Atmosphere: temperature, 20°±2° C.; booth air velocity, 0.3±0.1 m/second (push-pull downward flow)

(d) Setting time/temperature: 10 minutes/20°±2° C.

(e) Baking temperature/time: 140° C./25 minutes

Speed of elevating temperatures: 8 minutes from 20° C. to 140° C.

(f) Rotating conditions: The substrate to be rotated in parallel to its sides about a horizontal axis in 75 cm apart from the central axis thereof

For the setting step, the steel plate thus overcoated was then conveyed to a device as shown in FIG. 23 where a ultrasonic wave with a frequency of 23,000 Hz and an amplitude of 0.05 mm was applied. The application of the ultrasonic wave started in 3 minutes after the setting step started and continued for 20 seconds. During the application of the ultrasonic wave, the substrate was rotated at the rate of 30 rpm. The setting step is continued for 10 minutes, and thereafter the substrate was baked without application of the ultrasonic wave and rotation of the substrate.

FIG. 27(a) shows speeds of paint sagging when the ultrasonic wave was applied in the same conditions as above yet without rotation of the substrate during the application of the ultrasonic wave. For reference, the paint coated in the film thickness of 40  $\mu\text{m}$  was set and baked in the same manner as above as shown by the dashed line in FIG. 27(a), although no rotation was carried out.

Table 1 shows the results indicating the relationship of the film thicknesses vs. the speeds of rotation with the outside action applied during rotation. The values in the table are expressed in the PGD value. This is all the same for tables which follow.

TABLE 1

| Film Thickness ( $\mu\text{m}$ ) | Time of Vibration (sec) | Speed of Rotation (rpm) |     |     |     |     |
|----------------------------------|-------------------------|-------------------------|-----|-----|-----|-----|
|                                  |                         | 20                      | 25  | 30  | 35  | 40  |
| 20                               | 10                      | 0.4                     | 0.4 | 0.4 | 0.4 | 0.4 |

TABLE 1-continued

| Film Thickness<br>( $\mu$ m) | Time of Vibration<br>(sec) | Speed of Rotation (rpm) |     |     |     |       |
|------------------------------|----------------------------|-------------------------|-----|-----|-----|-------|
|                              |                            | 20                      | 25  | 30  | 35  | 40    |
| (0.3)                        | 20                         | 0.4                     | 0.4 | 0.4 | 0.4 | 0.4   |
|                              | 30                         | 0.4                     | 0.4 | 0.4 | 0.4 | 0.4   |
| 25                           | 10                         | 0.6                     | 0.6 | 0.6 | 0.6 | 0.6   |
| (0.4)                        | 20                         | 0.7                     | 0.7 | 0.7 | 0.7 | 0.7   |
|                              | 30                         | 0.7                     | 0.7 | 0.7 | 0.7 | 0.7   |
| 30                           | 10                         | SAG                     | 0.7 | 0.7 | 0.7 | 0.7   |
| (0.5)                        | 20                         | —                       | SAG | 0.8 | 0.8 | 0.8   |
|                              | 30                         | —                       | —   | 0.8 | 0.8 | 0.8   |
| 35                           | 10                         | SAG                     | SAG | 0.9 | 0.9 | SAG** |
| (0.6)                        | 20                         | —                       | —   | 1.0 | 1.0 | —     |
|                              | 30                         | —                       | —   | 1.0 | 1.0 | —     |

Notes:

(—)PGD value; without rotation and application of the outside action; vertical side finished

\*\*-Sagged in a reverse direction due to centrifugal force

## EXAMPLE 2

The steel plate was overcoated in varying film thicknesses as shown in Table 2 below and then treated in the same manner as in Example 1 with the exception that, in place of a ultrasonic wave, there was applied a vibration having a frequency of 240 Hz and an amplitude of 5.0 mm for three minutes in the setting step after 1 minute from the start of the setting step by traveling the carriage on wavy rails as shown in FIG. 20. During application of the vibration upwardly and downwardly in alternate directions, the rotation was carried out on the carriage at the rate of 15 rpm.

FIG. 27(b) shows speeds of paint sagging when the vibration was applied in the same conditions as above yet without rotation of the substrate during the application of the up-and-down vibration.

Table 2 shows the results indicating the relationship of the film thicknesses vs. the speeds of rotation with the outside action applied during rotation.

TABLE 2

| Film Thickness<br>( $\mu$ m) | Time of Vibration<br>(min) | Speed of Rotation (rpm) |     |     |     |     |
|------------------------------|----------------------------|-------------------------|-----|-----|-----|-----|
|                              |                            | 5                       | 10  | 15  | 20  | 25  |
| 20                           | 1                          | 0.3                     | 0.3 | 0.3 | 0.3 | 0.3 |
|                              | 3                          | 0.3                     | 0.3 | 0.3 | 0.3 | 0.3 |
|                              | 5                          | 0.3                     | 0.3 | 0.3 | 0.3 | 0.3 |
| 25                           | 1                          | 0.5                     | 0.5 | 0.5 | 0.5 | 0.5 |
|                              | 3                          | 0.5                     | 0.5 | 0.5 | 0.5 | 0.5 |
|                              | 5                          | 0.5                     | 0.5 | 0.5 | 0.5 | 0.5 |
| 30                           | 1                          | SAG                     | SAG | 0.6 | 0.6 | 0.6 |
|                              | 3                          | —                       | —   | 0.7 | 0.7 | 0.7 |
|                              | 5                          | —                       | —   | 0.7 | 0.7 | 0.7 |
| 35                           | 1                          | SAG                     | SAG | 0.8 | 0.8 | 0.8 |
|                              | 3                          | —                       | —   | 0.9 | 0.9 | 0.9 |
|                              | 5                          | —                       | —   | 0.9 | 0.9 | 0.9 |

## EXAMPLE 3

The steel plate was overcoated in varying film thicknesses as shown in Table 3 below and then treated in the same manner as in Example 2 with the exception that the same vibration was additionally applied for five minutes just after the start of the baking step in the same manner as in Example 2 while rotating the substrate at the rate of 15 rpm.

FIG. 27(c) shows speed of paint sagging when the vibration was applied in the same conditions as above

yet without rotation of the substrate during the application of the up-and-down vibration.

Table 3 shows the results indicating the relationship of the film thicknesses vs. the speeds of rotation with the outside action applied during rotation.

TABLE 3

| Time of Vibration<br>(minutes) | Setting<br>Step | Baking<br>Step | Speed of Rotation<br>(rpm) |     |     |     |     |
|--------------------------------|-----------------|----------------|----------------------------|-----|-----|-----|-----|
|                                |                 |                | 5                          | 10  | 15  | 20  | 25  |
| 10                             | 20              | 3              | 5                          | 0.3 | 0.3 | 0.3 | 0.3 |
|                                | 25              | 3              | 3                          | 0.5 | 0.5 | 0.5 | 0.5 |
|                                | 30              | 1              | 3                          | SAG | 0.6 | 0.6 | 0.6 |
| 15                             | 3               | 5              | —                          | 0.6 | 0.6 | 0.6 | 0.6 |
|                                | 3               | 3              | —                          | SAG | 0.8 | 0.8 | 0.8 |
|                                | 35              | 1              | 3                          | SAG | SAG | 0.8 | 0.8 |
| 20                             | 3               | 5              | —                          | —   | 0.8 | 0.8 | 0.8 |
|                                | 3               | 3              | —                          | —   | 0.8 | 0.8 | 0.8 |
|                                | 5               | —              | —                          | —   | 1.0 | 1.0 | 1.0 |

## EXAMPLE 4

The steel plate was overcoated in varying film thicknesses as shown in Table 4 below and then treated in the same manner as in Example 1 with the exception that, in place of application of a ultrasonic wave, the substrate was heated with a high-frequency wave using a device as shown in FIG. 18. The setting step was carried out at 20° C. for 3 minutes and then by elevating the temperature of the substrate from 20° C. to 60° C. in 30 seconds. The heating was kept at that temperature for 1.5 minutes and then allowed to cool. The substrate was rotated at 30 rpm for about two minutes while it was heated. After the setting step for 10 minutes, the substrate was then heated again to 140° C.

FIG. 27(d) shows speeds of paint sagging when the vibration was applied in the same conditions as above yet without rotation of the substrate during the application of the outside action.

Table 4 shows the results indicating the relationship of the film thicknesses vs. the speeds of rotation with the outside action applied during rotation.

TABLE 4

| Time of Heating<br>(min) | Setting<br>Step | Baking<br>Step | Speed of Rotation (rpm) |     |     |     |     |
|--------------------------|-----------------|----------------|-------------------------|-----|-----|-----|-----|
|                          |                 |                | 15                      | 20  | 25  | 30  | 35  |
| 50                       | 20              | 1              | 0.3                     | 0.3 | 0.3 | 0.3 | 0.3 |
|                          | 2               | 0.3            | 0.3                     | 0.3 | 0.3 | 0.3 | 0.3 |
|                          | 3               | 0.3            | 0.3                     | 0.3 | 0.3 | 0.3 | 0.3 |
| 55                       | 25              | 1              | 0.5                     | 0.5 | 0.5 | 0.5 | 0.5 |
|                          | 2               | 0.5            | 0.5                     | 0.5 | 0.5 | 0.5 | 0.5 |
|                          | 3               | 0.5            | 0.5                     | 0.5 | 0.5 | 0.5 | 0.5 |
| 60                       | 30              | 1              | 0.6                     | 0.6 | 0.6 | 0.6 | 0.6 |
|                          | 2               | SAG            | 0.8                     | 0.8 | 0.8 | 0.8 | 0.8 |
|                          | 3               | —              | 0.8                     | 0.8 | 0.8 | 0.8 | 0.8 |
| 65                       | 35              | 1              | SAG                     | 0.7 | 0.7 | 0.7 | 0.7 |
|                          | 2               | —              | 0.9                     | 0.9 | 0.9 | 0.9 | 0.9 |
|                          | 3               | —              | 0.9                     | 0.9 | 0.9 | 0.9 | 0.9 |

## EXAMPLE 5

The steel plate was overcoated in varying film thicknesses as shown in Table 5 below and then treated in the same manner as in Example 1 with the exception that, in place of application of a ultrasonic wave, the substrate was heated with infrared rays using a device as shown

in FIG. 17. The setting step was carried out at 20° C. for 1 minute and then by elevating the temperature of the substrate from 20° C. to 60° C. in one minute. The heating was kept at that temperature for three minutes and then allowed to cool. The substrate was rotated at 15 rpm for four minutes while it was heated. After the setting step for 10 minutes, the substrate was then heated again to 140° C.

FIG. 27(e) shows speeds of paint sagging when the vibration was applied in the same conditions as above yet without rotation of the substrate during the application of the outside action.

Table 5 shows the results indicating the relationship of the film thicknesses vs. the speeds of rotation with the outside action applied during rotation.

TABLE 5

| Film Thickness (μm) | Time of Heating (min) | Speed of Rotation (rpm) |     |     |     |     |
|---------------------|-----------------------|-------------------------|-----|-----|-----|-----|
|                     |                       | 5                       | 10  | 15  | 20  | 25  |
| 20                  | 2                     | 0.3                     | 0.3 | 0.3 | 0.3 | 0.3 |
|                     | 4                     | 0.3                     | 0.3 | 0.3 | 0.3 | 0.3 |
|                     | 6                     | 0.3                     | 0.3 | 0.3 | 0.3 | 0.3 |
| 25                  | 2                     | 0.5                     | 0.5 | 0.5 | 0.5 | 0.5 |
|                     | 4                     | 0.5                     | 0.5 | 0.5 | 0.5 | 0.5 |
|                     | 6                     | 0.5                     | 0.5 | 0.5 | 0.5 | 0.5 |
| 30                  | 2                     | SAG                     | 0.7 | 0.7 | 0.7 | 0.7 |
|                     | 4                     | —                       | 0.7 | 0.7 | 0.7 | 0.7 |
|                     | 6                     | —                       | 0.7 | 0.7 | 0.7 | 0.7 |
| 35                  | 2                     | —                       | 0.9 | 0.9 | 0.9 | 0.9 |
|                     | 4                     | —                       | 0.9 | 0.9 | 0.9 | 0.9 |
|                     | 6                     | —                       | 0.9 | 0.9 | 0.9 | 0.9 |

## EXAMPLE 6

The steel plate was overcoated in varying film thicknesses as shown in Table 6 below and then treated in the same manner as in Example 1 with the exception that, in place of application of a ultrasonic wave, the substrate was heated with hot air using a device as shown in FIG. 19. The setting step was carried out at 20° C. for 1 minute and then by elevating the temperature of the substrate from 20° C. to 60° C. in three minutes. The heating was kept at that temperature for one minute and then allowed to cool. The substrate was rotated at 10 rpm for four minutes while it was heated. After the setting step for 10 minutes, the substrate was then heated again to 140° C.

FIG. 27(f) shows speeds of paint sagging when the vibration was applied in the same conditions as above yet without rotation of the substrate during the application of the outside action.

Table 6 shows the results indicating the relationship of the film thicknesses vs. the speeds of rotation with the outside action applied during rotation.

TABLE 6

| Film Thickness (μm) | Time of Heating (min) | Speed of Rotation (rpm) |     |     |     |     |
|---------------------|-----------------------|-------------------------|-----|-----|-----|-----|
|                     |                       | 5                       | 10  | 15  | 20  | 25  |
| 20                  | 4                     | 0.3                     | 0.3 | 0.3 | 0.3 | 0.3 |
|                     | 6                     | 0.3                     | 0.3 | 0.3 | 0.3 | 0.3 |
|                     | 8                     | 0.3                     | 0.3 | 0.3 | 0.3 | 0.3 |
| 25                  | 4                     | 0.5                     | 0.5 | 0.5 | 0.5 | 0.5 |
|                     | 6                     | 0.5                     | 0.5 | 0.5 | 0.5 | 0.5 |
|                     | 8                     | 0.5                     | 0.5 | 0.5 | 0.5 | 0.5 |
| 30                  | 4                     | 0.7                     | 0.7 | 0.7 | 0.7 | 0.7 |
|                     | 6                     | 0.7                     | 0.7 | 0.7 | 0.7 | 0.7 |

TABLE 6-continued

| Film Thickness (μm) | Time of Heating (min) | Speed of Rotation (rpm) |     |     |     |     |
|---------------------|-----------------------|-------------------------|-----|-----|-----|-----|
|                     |                       | 5                       | 10  | 15  | 20  | 25  |
| 35                  | 8                     | 0.7                     | 0.7 | 0.7 | 0.7 | 0.7 |
|                     | 4                     | 0.9                     | 0.9 | 0.9 | 0.9 | 0.9 |
|                     | 6                     | 0.9                     | 0.9 | 0.9 | 0.9 | 0.9 |
|                     | 8                     | 0.9                     | 0.9 | 0.9 | 0.9 | 0.9 |

## EXAMPLE 7

A cold rolled steel plate was overcoated in varying film thicknesses as shown in Table 7 below in the same manner as in Example 1 using a two-component liquid urethane paint with the exception of treating conditions as follows:

- (a) Paint:
  - (i) Main agent: acrylic resin (black; average weight, 2,500)
  - (ii) Curing agent: polyisocyanate
  - (iii) Ratio of main agent to curing agent: 7 to 1
  - (iv) Viscosity of spraying: 16 seconds (when measured by Ford Cup #4 at 20° C., without a sag preventing agent)
  - (v) Unvolatilizables: 54% by weight
  - (vi) Solvent: ethyl acetate, 15 parts by weight, butyl acetate, 55 parts by weight, Cellosolve acetate, 30 parts by weight

(b) Coating and drying conditions: The same as in Example 1 except the baking step carried out at 90° C. for 25 minutes with the temperature accelerated from 20° C. to 90° C. in 5 minutes

(c) Film thickness at sagging limit: 45 μm  
The substrate overcoated above was then tested for its coating performance in substantially the same manner as in Example 1.

FIG. 28(a) shows speeds of paint sagging when the vibration was applied in the same conditions as above yet without rotation of the substrate during the application of the outside action. In FIG. 28(a), the dashed line indicates a coating in a film thickness of 45 μm which was set and baked without application of the outside action and rotation.

Table 7 shows the results indicating the relationship of the film thicknesses vs. the speeds of rotation with the outside action applied during rotation.

TABLE 7

| Film Thickness (μm) | Time of Vibration (sec) | Speed of Rotation (rpm) |     |     |     |     |
|---------------------|-------------------------|-------------------------|-----|-----|-----|-----|
|                     |                         | 10                      | 15  | 20  | 25  | 30  |
| 25                  | 10                      | 0.5                     | 0.5 | 0.5 | 0.5 | 0.5 |
|                     | 20                      | 0.5                     | 0.5 | 0.5 | 0.5 | 0.5 |
|                     | 30                      | 0.5                     | 0.5 | 0.5 | 0.5 | 0.5 |
|                     | 40                      | 0.6                     | 0.6 | 0.6 | 0.6 | 0.6 |
|                     | 50                      | 0.6                     | 0.6 | 0.6 | 0.6 | 0.6 |
|                     | 60                      | 0.6                     | 0.6 | 0.6 | 0.6 | 0.6 |
|                     | 70                      | 0.7                     | 0.7 | 0.7 | 0.7 | 0.7 |
|                     | 80                      | —                       | —   | 0.9 | 0.9 | 0.9 |
|                     | 90                      | —                       | —   | 0.9 | 0.9 | 0.9 |
|                     | 100                     | —                       | —   | 1.0 | 1.0 | 1.0 |
| 35                  | 10                      | SAG                     | SAG | 0.7 | 0.7 | 0.7 |
|                     | 20                      | —                       | —   | 0.9 | 0.9 | 0.9 |
|                     | 30                      | —                       | —   | 0.9 | 0.9 | 0.9 |
|                     | 40                      | SAG                     | SAG | SAG | 0.9 | 0.9 |
|                     | 50                      | —                       | —   | —   | 1.0 | 1.0 |

Notes:  
(-) PGD value; without rotation and application of the outside action; vertical side finished

## EXAMPLE 8

The steel plate was overcoated in varying film thicknesses as shown in Table 8 below and then treated in the same manner as in Example 2 with the exception that, in place of a ultrasonic wave, there was applied a vibration having a frequency of 240 Hz and an amplitude of 5.0 mm for three minutes in the setting step after 1 minute from the start of the setting step by traveling the carriage on wavy rails as shown in FIG. 20. During application of the vibration upwardly and downwardly in alternate directions, the rotation was carried out at the rate of 15 rpm.

FIG. 28(b) shows speeds of paint sagging when the vibration was applied in the same conditions as above yet without rotation of the substrate during the application of the up-and-down vibration.

Table 8 shows the results indicating the relationship of the film thicknesses vs. the speeds of rotation with the outside action applied during rotation.

TABLE 8

| Film Thickness<br>( $\mu$ m) | Time of Vibration<br>(min) | Speed of Rotation (rpm) |     |     |     |     |
|------------------------------|----------------------------|-------------------------|-----|-----|-----|-----|
|                              |                            | 10                      | 15  | 20  | 25  | 30  |
| 25                           | 1                          | 0.4                     | 0.4 | 0.4 | 0.4 | 0.4 |
|                              | 3                          | 0.5                     | 0.5 | 0.5 | 0.5 | 0.5 |
|                              | 5                          | 0.5                     | 0.5 | 0.5 | 0.5 | 0.5 |
| 30                           | 1                          | 0.5                     | 0.5 | 0.5 | 0.5 | 0.5 |
|                              | 3                          | 0.6                     | 0.6 | 0.6 | 0.6 | 0.6 |
|                              | 5                          | 0.6                     | 0.6 | 0.6 | 0.6 | 0.6 |
| 35                           | 1                          | 0.7                     | 0.7 | 0.7 | 0.7 | 0.7 |
|                              | 3                          | 0.9                     | 0.9 | 0.9 | 0.9 | 0.9 |
|                              | 5                          | 0.9                     | 0.9 | 0.9 | 0.9 | 0.9 |
| 40                           | 1                          | SAG                     | 0.9 | 0.9 | 0.9 | 0.9 |
|                              | 3                          | —                       | 1.0 | 1.0 | 1.0 | 1.0 |
|                              | 5                          | —                       | 1.0 | 1.0 | 1.0 | 1.0 |

## EXAMPLE 9

The steel plate was overcoated in varying film thicknesses as shown in Table 9 below and then treated in the same manner as in Example 4 with the exception that, in place of application of a ultrasonic wave, the substrate was heated with a high-frequency wave. The setting step was carried out by placing the substrate in a device as shown in FIG. 18 at 20° C. for 3 minutes and then by elevating the temperature of the substrate to 60° C. in 30 seconds. The heating was kept at that temperature for 1.5 minutes and then allowed to cool. The substrate was rotated in 30 rpm for about two minutes while it was heated. After the setting step for 10 minutes, the substrate was then heated again to 140° C.

FIG. 28(c) shows speeds of paint sagging when the vibration was applied in the same conditions as above yet without rotation of the substrate during the application of the outside action.

Table 9 shows the results indicating the relationship of the film thicknesses vs. the speeds of rotation with the outside action applied during rotation.

TABLE 9

| Film Thickness<br>( $\mu$ m) | Time of Heating<br>(min) | Speed of Rotation (rpm) |     |     |     |     |
|------------------------------|--------------------------|-------------------------|-----|-----|-----|-----|
|                              |                          | 10                      | 15  | 20  | 25  | 30  |
| 25                           | 1                        | 0.4                     | 0.4 | 0.4 | 0.4 | 0.4 |
|                              | 2                        | 0.4                     | 0.4 | 0.4 | 0.4 | 0.4 |

TABLE 9-continued

| 5  | Film Thick-<br>ness<br>( $\mu$ m) | Time<br>of<br>Heat-<br>ing<br>(min) | Speed of Rotation (rpm) |     |     |     |     |
|----|-----------------------------------|-------------------------------------|-------------------------|-----|-----|-----|-----|
|    |                                   |                                     | 10                      | 15  | 20  | 25  | 30  |
| 10 | 30                                | 3                                   | 0.4                     | 0.4 | 0.4 | 0.4 | 0.4 |
|    |                                   | 1                                   | 0.6                     | 0.6 | 0.6 | 0.6 | 0.6 |
|    |                                   | 2                                   | 0.6                     | 0.6 | 0.6 | 0.6 | 0.6 |
| 15 | 35                                | 3                                   | 0.6                     | 0.6 | 0.6 | 0.6 | 0.6 |
|    |                                   | 1                                   | 0.7                     | 0.7 | 0.7 | 0.7 | 0.7 |
|    |                                   | 2                                   | 0.7                     | 0.7 | 0.7 | 0.7 | 0.7 |
| 15 | 40                                | 3                                   | 0.7                     | 0.7 | 0.7 | 0.7 | 0.7 |
|    |                                   | 1                                   | SAG                     | SAG | 0.9 | 0.9 | 0.9 |
|    |                                   | 2                                   | —                       | —   | 0.9 | 0.9 | 0.9 |
|    |                                   | 3                                   | —                       | —   | 0.9 | 0.9 | 0.9 |

## EXAMPLE 10

The steel plate was overcoated in varying film thicknesses as shown in Table 10 below and then treated in the same manner as in Example 7 with the exception that, in place of application of a ultrasonic wave, the substrate was heated with infrared rays using a device as shown in FIG. 18. The setting step was carried out at 20° C. for one minute and then by elevating the temperature of the substrate from 20° C. to 60° C. in one minute. The heating was kept at that temperature for 1.5 minutes and then allowed to cool. The substrate was rotated at 15 rpm for four minutes while it was heated.

30 After the setting step for 10 minutes, the substrate was then heated again to 140° C.

FIG. 28(d) shows speeds of paint sagging when the vibration was applied in the same conditions as above yet without rotation of the substrate during the application of the outside action.

Table 10 shows the results indicating the relationship of the film thicknesses vs. the speeds of rotation with the outside action applied during rotation.

TABLE 10

| 40 | Film Thick-<br>ness<br>( $\mu$ m) | Time<br>of<br>Heat-<br>ing<br>(min) | Speed of Rotation (rpm) |     |     |     |     |
|----|-----------------------------------|-------------------------------------|-------------------------|-----|-----|-----|-----|
|    |                                   |                                     | 10                      | 15  | 20  | 25  | 30  |
| 45 | 25                                | 2                                   | 0.5                     | 0.5 | 0.5 | 0.5 | 0.5 |
|    |                                   | 4                                   | 0.5                     | 0.5 | 0.5 | 0.5 | 0.5 |
|    |                                   | 6                                   | 0.5                     | 0.5 | 0.5 | 0.5 | 0.5 |
| 50 | 30                                | 2                                   | 0.6                     | 0.6 | 0.6 | 0.6 | 0.6 |
|    |                                   | 4                                   | 0.6                     | 0.6 | 0.6 | 0.6 | 0.6 |
|    |                                   | 6                                   | 0.6                     | 0.6 | 0.6 | 0.6 | 0.6 |
| 55 | 35                                | 2                                   | 0.7                     | 0.7 | 0.7 | 0.7 | 0.7 |
|    |                                   | 4                                   | 0.9                     | 0.9 | 0.9 | 0.9 | 0.9 |
|    |                                   | 6                                   | 0.9                     | 0.9 | 0.9 | 0.9 | 0.9 |
|    | 40                                | 2                                   | SAG                     | 0.9 | 0.9 | 0.9 | 0.9 |
|    |                                   | 4                                   | —                       | 1.0 | 1.0 | 1.0 | 1.0 |
|    |                                   | 6                                   | —                       | 1.0 | 1.0 | 1.0 | 1.0 |

## EXAMPLE 11

The steel plate was overcoated in varying film thicknesses as shown in Table 11 below and then treated in the same manner as in Example 7 with the exception that, in place of application of a ultrasonic wave, the substrate was heated with hot air using a device as shown in FIG. 19. The setting step was carried out at 20° C. for one minute and then by elevating the temperature of the substrate from 20° C. to 60° C. in three minutes. The heating was kept at that temperature for one minute and then allowed to cool. The substrate was

rotated at 10 rpm for about four minutes while it was heated. After the setting step for 10 minutes, the substrate was then heated again to 140° C.

FIG. 28(e) shows speeds of paint sagging when the vibration was applied in the same conditions as above yet without rotation of the substrate during the application of the outside action. Table 11 shows the results indicating the relationship of the film thicknesses vs. the speeds of rotation with the outside action applied during rotation.

TABLE 11

| Film Thickness<br>( $\mu$ m) | Time of Heating<br>(min) | Speed of Rotation (rpm) |     |     |     |     |
|------------------------------|--------------------------|-------------------------|-----|-----|-----|-----|
|                              |                          | 10                      | 15  | 20  | 25  | 30  |
| 25                           | 2                        | 0.5                     | 0.5 | 0.5 | 0.5 | 0.5 |
|                              | 4                        | 0.5                     | 0.5 | 0.5 | 0.5 | 0.5 |
|                              | 6                        | 0.5                     | 0.5 | 0.5 | 0.5 | 0.5 |
| 30                           | 2                        | 0.6                     | 0.6 | 0.6 | 0.6 | 0.6 |
|                              | 4                        | 0.6                     | 0.6 | 0.6 | 0.6 | 0.6 |
|                              | 6                        | 0.6                     | 0.6 | 0.6 | 0.6 | 0.6 |
| 35                           | 2                        | 0.7                     | 0.7 | 0.7 | 0.7 | 0.7 |
|                              | 4                        | 0.9                     | 0.9 | 0.9 | 0.9 | 0.9 |
|                              | 6                        | 0.9                     | 0.9 | 0.9 | 0.9 | 0.9 |
| 40                           | 2                        | SAG                     | 0.9 | 0.9 | 0.9 | 0.9 |
|                              | 4                        | SAG                     | 1.0 | 1.0 | 1.0 | 1.0 |
|                              | 6                        | SAG                     | 1.0 | 1.0 | 1.0 | 1.0 |

## EXAMPLE 12

A cold rolled steel plate was undercoated and then intercoated in substantially the same manner as in Example 1.

The plate so intercoated was then overcoated with a powder paint in varying film thicknesses as shown in Table 12 and baked in substantially the same manner as in Example 1 unless otherwise stated hereinbelow:

(a) Paint: Acrylic powder paint (average molecular weight: 4,000; black)

(b) Powder spray gun by electrodeposition: 1 stage coating on a surface extending vertically

(c) Baking temperature/time: 150° C./20 minutes; accelerated from 20° C. to 150° C. in 10 minutes

(d) Film thickness at sagging threshold value: 100  $\mu$ m

The substrate was subjected to a vibration by applying an ultrasonic wave with a frequency of 23,000 Hz and an amplitude of 0.05 mm was applied after one minute from the start of the baking step. During the application of the ultrasonic wave, the substrate was rotated at the rate of 20 rpm.

FIG. 29(a) shows speeds of paint sagging when the ultrasonic wave was applied in the same conditions as above yet without rotation of the substrate during the application of the ultrasonic wave. As shown in FIG. 27(a), the paint was coated in the film thickness of 100  $\mu$ m and baked in the same manner as hereinabove, although no rotation was carried out.

Table 12 shows the results indicating the relationship of the film thicknesses vs. the speeds of rotation with the outside action applied during rotation.

It is to be noted herein that the use of powder paints as in this embodiment does not require the setting step so that a substrate coated with powder paints may be conveyed directly to the baking step from the coating step.

TABLE 12

| Film Thickness<br>( $\mu$ m) | Time of Vibration<br>(sec) | Speed of Rotation (rpm) |     |     |     |     |
|------------------------------|----------------------------|-------------------------|-----|-----|-----|-----|
|                              |                            | 10                      | 15  | 20  | 25  | 30  |
| 5                            | 60<br>(0.1)                | 0.1                     | 0.1 | 0.1 | 0.1 | 0.1 |
|                              | 60                         | 0.1                     | 0.1 | 0.1 | 0.1 | 0.1 |
|                              | 90                         | 0.1                     | 0.1 | 0.1 | 0.1 | 0.1 |
|                              | 70<br>(0.3)                | 0.3                     | 0.3 | 0.3 | 0.3 | 0.3 |
|                              | 60                         | 0.4                     | 0.4 | 0.4 | 0.4 | 0.4 |
|                              | 90                         | 0.4                     | 0.4 | 0.4 | 0.4 | 0.4 |
|                              | 80<br>(0.4)                | 0.5                     | 0.5 | 0.5 | 0.5 | 0.5 |
|                              | 60                         | 0.7                     | 0.7 | 0.7 | 0.7 | 0.7 |
|                              | 90                         | 0.7                     | 0.7 | 0.7 | 0.7 | 0.7 |
|                              | 90<br>(0.5)                | SAG                     | 0.8 | 0.8 | 0.8 | 0.8 |
| 10                           | 60                         | —                       | SAG | 0.9 | 0.9 | 0.9 |
|                              | 90                         | —                       | —   | 0.9 | 0.9 | 0.9 |

## Notes:

(-)PGD value; without rotation and application of the outside action; vertical side finished

20

## EXAMPLE 13

The steel plate was overcoated in varying film thicknesses as shown in Table 13 below and then treated in the same manner as in Example 12 with the exception that, in place of a ultrasonic wave, there was applied a vibration having a frequency of 240 Hz and an amplitude of 5.0 mm for three minutes in the baking step after five minutes from the start of the baking step by traveling the carriage on wavy rails as shown in FIG. 20. During application of the vibration upwardly and downwardly in alternate directions, the rotation was carried out at the rate of 15 rpm.

FIG. 29(b) shows speeds of paint sagging when the vibration was applied in the same conditions as above yet without rotation of the substrate during the application of the up-and-down vibration.

Table 13 shows the results indicating the relationship of the film thicknesses vs. the speeds of rotation with the outside action applied during rotation.

TABLE 13

| Film Thickness<br>( $\mu$ m) | Time of Vibration<br>(min) | Speed of Rotation (rpm) |     |     |     |     |
|------------------------------|----------------------------|-------------------------|-----|-----|-----|-----|
|                              |                            | 10                      | 15  | 20  | 25  | 30  |
| 45                           | 60                         | 0.1                     | 0.1 | 0.1 | 0.1 | 0.1 |
|                              | 3                          | 0.1                     | 0.1 | 0.1 | 0.1 | 0.1 |
|                              | 5                          | 0.1                     | 0.1 | 0.1 | 0.1 | 0.1 |
|                              | 70                         | 0.3                     | 0.3 | 0.3 | 0.3 | 0.3 |
|                              | 3                          | 0.4                     | 0.4 | 0.4 | 0.4 | 0.4 |
|                              | 5                          | 0.4                     | 0.4 | 0.4 | 0.4 | 0.4 |
|                              | 80                         | 0.6                     | 0.6 | 0.6 | 0.6 | 0.6 |
|                              | 3                          | 0.7                     | 0.7 | 0.7 | 0.7 | 0.7 |
|                              | 5                          | 0.7                     | 0.7 | 0.7 | 0.7 | 0.7 |
|                              | 90                         | 0.8                     | 0.8 | 0.8 | 0.8 | 0.8 |
| 55                           | 3                          | SAG                     | 1.0 | 1.0 | 1.0 | 1.0 |
|                              | 5                          | —                       | 1.0 | 1.0 | 1.0 | 1.0 |

It is to be understood that the foregoing text and drawings relates to embodiments of the present invention given by way of examples but not limitations. Various other embodiments and variants are possible within the spirit and scope of the present invention.

What is claimed is:

1. A coating method comprising:  
a coating step for spraying a surface of a substrate with a paint; and  
a drying step for drying the paint sprayed on the surface of the substrate;

wherein the paint is sprayed during the coating step to form a coating a film thickness which is thinner than a thickness at which the coat begins to sag in either the coating step or the drying step; wherein an action is applied from outside the substrate in at least one of the coating and drying steps so as to cause the paint coated on the substrate to flow or sag in the drying step; and wherein the substrate is rotated about an axis extending substantially horizontally in a longitudinal direction of the substrate while the paint of the coat flows as a result of the application of the action from the outside at a speed which is high enough to rotate the substrate before the paint of the coat substantially sags due to gravity yet which is low enough so as to cause no sagging as a result of centrifugal force.

2. A coating method as claimed in claim 1, wherein the drying step comprises a setting step and a baking step and an ambient temperature in the setting step is lower than the temperature during the baking step.

3. A coating method as claimed in claim 2, wherein the action is applied by heating the paint coated thereon in the setting step.

4. A coating method as claimed in claim 3, where the heating is effected from the inside of the substrate.

5. A coating method as claimed in claim 3, wherein the paint coated thereon is heated at an ambient temperature higher than the temperature set in the setting step.

6. A coating method as claimed in claim 3, wherein the heating is effected by an infrared panel.

7. A coating method as claimed in claim 3, wherein the heating is effected by a high-frequency induction coil.

8. A coating method as claimed in claim 4, wherein the action is applied by feeding hot air toward inside the substrate.

9. A coating method as claimed in claim 2, wherein no rotation of the substrate is carried out in the baking step.

10. A coating method as claimed in claim 2, wherein the rotation of the substrate is carried out in the baking step.

11. A coating method as claimed in claim 2, wherein a paint is a thermosetting paint containing a solvent.

12. A coating method as claimed in claim 1, wherein the rotation of the substrate is carried out intermittently.

13. A coating method as claimed in claim 1, wherein the action is a vibration during the drying step applied within the paint coated on the substrate.

14. A coating method as claimed in claim 13, wherein the drying step comprises setting and baking steps, and an ambient temperature in the setting step is set to be lower than the ambient temperature during the baking step.

15. A coating method as claimed in claim 14, wherein the vibration is produced both in the setting and baking steps.

16. A coating method as claimed in claim 13, wherein the vibration is produced in upward and downward directions.

17. A coating method as claimed in claim 13, wherein the vibration is produced acoustically.

18. A coating method as claimed in claim 1, wherein the coating substrate is a vehicle body.

19. A coating method as claimed in claim 18, wherein the horizontal axis of the body is set to extend horizontally in a longitudinal direction thereof.

20. A coating method as claimed in claim 2, wherein the horizontal axis is set to pass through the center of gravity of the coating substrate.

21. A coating method as claimed in claim 1, wherein the paint is a thermosetting paint.

22. A coating method as claimed in claim 1, wherein the rotation of the substrate is carried out continuously in one predetermined direction.

23. A coating method as claimed in claim 1, wherein the rotation of the substrate is carried out alternatively first in one direction and then in the opposite direction.

24. A coating method as claimed in claim 13, wherein the paint is dried in the drying step while the substrate is conveyed by a conveyance means; and the conveyance means is provided with a vibration-applying means for applying a vibration as an action from outside.

25. A coating method as claimed in claim 14, wherein the vibration is applied in the setting step alone.

26. A coating method as claimed in claim 25, wherein the paint is a two-component curing paint comprising a major component and a curing agent.

27. A coating method as claimed in claim 14, wherein the vibration is applied in the baking step alone.

28. A coating method as claimed in claim 27, wherein the paint is a powder paint.

\* \* \* \* \*